

# United States Patent

Tatchell

[15] 3,663,170

[45] May 16, 1972

[54] **MANUFACTURE OF CARBON FILAMENTS**

[72] Inventor: **John J. Tatchell**, Maidenstone, Kent, England

[73] Assignee: **Morganite Research & Development Limited**, London, England

[22] Filed: **Jan. 31, 1969**

[21] Appl. No.: **795,719**

[30] **Foreign Application Priority Data**

Feb. 21, 1968 Great Britain ..... 5,354/68

[52] U.S. Cl. .... **23/209.4, 23/209.1, 264/29**

[51] Int. Cl. .... **C01b 31/07**

[58] **Field of Search** ..... 23/209.1, 209.2, 209.4; 264/29

[56] **References Cited**

UNITED STATES PATENTS

3,285,696 11/1966 Tsunoda ..... 23/209.1

3,412,062 11/1968 Johnson et al. .... 260/37

*Primary Examiner*—Edward J. Meros  
*Attorney*—Plumley, Tyner & Sandt

[57] **ABSTRACT**

A process is disclosed for the production of carbon filaments having a very high modulus of elasticity which have utility as structural materials.

The process comprises the carbonization and pyrolysis of a filamentary material capable of carbonization with maintenance of its filamentary structure to temperatures above 900° C in which the filamentary material is a multifilament tow and this is heated up to a temperature of at least about 900° C under conditions of imposed linearity to reduce incidence of kinks in the carbon filaments. The linearity is preferably imposed by imparting a twist to the tow. A preferred raw material is a multifilament tow of a polyacrylonitrile polymer or copolymer containing at least 85% of acrylonitrile. The carbon filaments produced by the process of the invention have a reduced incidence of kinks.

**3 Claims, No Drawings**

## MANUFACTURE OF CARBON FILAMENTS

## BACKGROUND OF INVENTION

This invention relates to the production of carbon filaments having a very high modulus of elasticity.

Carbon filaments having a very high modulus of elasticity, for example above  $20 \times 10^6$  p.s.i. and an ultimate tensile strength above 150,000 p.s.i. are known and are capable of important use as structural materials when incorporated in matrices such as plastics and metal.

The starting material for the production of such carbon filaments is essentially a filamentary metal capable of carbonization without destruction of its filamentary nature. Organic materials which may be used for this purpose include natural and synthetic cellulose, which term include esters and ethers of cellulose, and polymers or co-polymer of acrylonitrile. The steps in the production of the filament include in general a controlled pyrolysis step to form the carbonaceous material and a subsequent step of heating to well above the pyrolysis temperature.

In one process of this type a cellulosic material is subjected to a carefully controlled heating schedule in a protected atmosphere. This schedule has the aim of raising the temperature slowly from room temperature to about 400° C to decompose the chemical structure of the cellulosic material without destroying its filamentary nature, then somewhat quicker increase of temperature up to about 900° C to remove further more stable constituents of the pyrolyzed material and produce a filament component substantially of carbon, and finally a rapid heating up to about 3000° C to complete the pyrolysis and generate a stable carbon filament which may contain graphitic constituents.

In another process of this type a polymer or co-polymer of acrylonitrile preferably containing at least 85 mole per cent of acrylonitrile is wound on a frame and heated in the presence of oxygen at 190°-260° C to modify the chemical structure of the polymer and form a blackened filament which can then be pyrolyzed by subsequent heating in a protective atmosphere, for example argon, up to about 3,000° C to form a stable carbon filament which may contain graphitic constituents. This subsequent heating may take place in two stages the first involving heating to about 900°-1500° C to produce a product of high strength the second optional heating stage being heating to about 3000° C to produce a product of high modulus but somewhat lower strength than that product which results from the first heating stage.

One difficulty which occurs in the production of carbon filaments by the process outlined above is the production of kink free filaments. The production of such filaments is highly desirable because of the application of the material as a structural reinforcing element. This is because the full benefit of the high strength and high modulus properties of the filaments is obtained primarily under direct tensile loading of the filaments and is obtained relatively poorly if the filaments are oriented so that portions thereof lie across the direction of the forces loading the structural component.

The defects in the linearity of the carbon filaments which most commonly occur are in the form of bends or kinks of about one-fourth inch in length and it is an object of the present invention to provide a process for the production of carbon filaments having a reduced incidence of defects in linearity, in order to realize fully the inherent physical properties of such materials.

We have found that this may be achieved by carrying out the heating of the carbonaceous material forming the filaments under conditions which impose a linearity on the material up to temperature of at least about 900° C. Thereafter the dimensional changes are relatively small and there is only a small chance of bends or kinks developing. This is achieved for example where the raw material is a multi-filament tow of polyacrylonitrile by imparting radial compression of the filaments with respect to the longitudinal axis of the tow during the heating in the presence of oxygen to modify the

chemical structure so as to bond the filaments together and to continue the heating of the filaments to a temperature of about 900° C with the filaments bonded together in this manner. It is found that at the end of this treatment step the individual filaments are substantially free of bends and kinks and may be separated one from the other.

Accordingly the invention provides a process for the production of carbon filaments by the carbonization and pyrolysis of a filamentary material capable of carbonization with maintenance of its filamentary structure to temperatures above 900° C in which the filamentary material is a multifilament tow and this is heated up to a temperature of at least about 900° C under conditions of imposed linearity to reduce incidence of kinks in the carbon filaments.

The radial compression can be imparted to the multi-filament tow in any suitable manner and may to some extent be inherent in the raw material. One method by which radial compression may be imposed is by imparting a controlled twist to the tow which causes the outer filaments to exert a radial compression on the inner filaments. A twist within the range of one twist per every 6 inches to every 2 feet is preferred and in practice a twist of about one twist per foot has been found to be advantageous. Other methods which may be used in combination therewith are carrying the decomposition out under tension and restricting the shrinkage of the material at this stage.

When the organic raw material, that is the multi-filament tow is modified by heating adherence takes place between the carbonaceous filaments. The radial compression on the material can then be released because linearity is still imposed on the carbon filaments by the adherence of the filaments to each other. When treatment of this material by heating to at least 900° C is continued the position of each filament is fixed with respect to each other so the incidence of bends and kinks in the individual filaments is reduced. After the heating treatment is complete the filaments may be separated from the filament bundle and are substantially free of kinks. They may if desired be further processed by the process described in the application of even date herewith of Kenneth G.O. Dixon et al entitled "Improvements in or Relating to the Manufacture of Filamentary Materials" by heating to a much higher temperature in conditions where oxygen and active materials are eliminated from the environment of the filament.

A preferred raw material for carrying out the process of the present invention is polyacrylonitrile polymer or copolymer in the form of a multi-filament tow. Decomposition of which is preferably effected by heating it at approximately 220° C in the presence of oxygen under tension and with an imparted twist. The invention is particularly applicable to the production of carbon filaments having a length in excess of 18 inches.

In order that the invention may be more fully understood, the following example is given, by way of illustration only:

55

## EXAMPLE

A polymeric filament being a co-polymer of 93 weight percent acrylonitrile, 6 weight percent methyl methacrylate and 1 weight percent itaconic acid, each filament being 1.5 denier and having a tenacity of not less than 5.5 grams per denier, the filaments being contained in a tow containing 10,000 filaments approximately was wound on a metal frame and heated in the presence of an oxygen containing atmosphere at 220° C to modify the chemical structure of the polymeric material. The color of the material after heating was black. During this heating stage, radial compression was obtained by applying a tension of about 2 kilograms while winding the material onto the frame, by restricting the shrinkage of the material during this heating stage thereby increasing the tension sharply as volatile products are driven off, and by giving individual filaments a helical configuration longitudinally of the tow, for example by giving the tow one twist every 12 inches.

The blackened filaments were cut off the frames in lengths of 1 meter and were transferred very carefully, retaining the

adhesion between individual filaments, to a carbon boat. This stage is critical because any bending of the blackened tow can destroy the adhesion between the filaments. The carbon boat was filled with a large number of such lengths arranged very carefully parallel to each other and retained in the boat under slight compression of about 1 kilogram obtained by means of a carbon lid.

The boat was transferred to an oven and heated to a temperature of 1,000° C in a protective atmosphere of nitrogen. Heating was continued until evolution of cracked products had ceased.

The material so obtained had a diameter of 7 microns, a modulus of  $28 \times 10^6$  p.s.i. and an ultimate tensile strength of 260,000 p.s.i. The product was substantially straight and free from kinks and could be handled quite freely for incorporation into a structural matrix.

I claim:

1. A process for the production of carbon filaments which comprises the steps of heating a multi-filament polyacrylonitrile tow to a temperature of 190°-260° C in the presence of oxygen to modify the filaments, said heating being carried out on the material while it is under tension and after a controlled twist within the range of one twist per every 6 inches to 2 feet has been imparted thereto so as to impart radial compression to the filaments with respect to the longitudi-

25

dinal axis of the tow and cause the filaments to adhere together and transferring the modified filaments to a heating zone and heating to a temperature of at least about 900° C in an atmosphere free of oxygen, care being taken during said

5 transfer to maintain the adhesion between the filaments.

2. A process as claimed in 1 in which a twist of about one twist per foot has been imparted to the material.

3. A process for the production of carbon filaments which comprises the steps of heating a multifilament polyacrylonitrile tow to a temperature of 190°-260° C in the presence of oxygen to modify the filaments, said heating being carried on the material while it is under tension and after a controlled twist within the range of one twist per every 6 inches to 2 feet has been imparted thereto so as to impart radial compression to the filaments with respect to the longitudinal axis of the tow and cause the filaments to adhere together and transferring the modified filaments to a heating zone, and heating said modified filaments in an atmosphere free of oxygen to a temperature of at least about 900° C, care being taken during said transfer to maintain the adhesion between the filaments, and heating said resulting filaments to a temperature substantially in excess of 900° C in the presence of a carbon gettering material.

\* \* \* \* \*

30

35

40

45

50

55

60

65

70

75